

## UNITED STATES PATENT OFFICE

2,245,876

## MALLEABLE IRON PROCESS

Harry A. Schwartz, Cleveland Heights, Ohio, assignor to National Malleable and Steel Castings Company, Cleveland, Ohio, a corporation of Ohio

No Drawing. Application February 15, 1940,  
Serial No. 319,105

6 Claims. (Cl. 148—3)

This invention relates to a process for reducing the annealing time of white cast iron when converting it to malleable iron and in improving the physical properties of the resulting malleable iron. More particularly the invention concerns the improvement of said physical properties and annealing time by a reduction of the moisture in the air blast used in the melting furnace.

It has been observed on different occasions that the physical properties of malleable iron varied considerably even when made by the same process and when the usual analysis showed no substantial difference in the generally accepted variables. During an investigation into the cause of this behavior of the metal I discovered that the hydrogen in the white cast iron, although present in minute quantities, varied in some specimens by several hundred percent over that in other specimens. Correlation of the hydrogen in a series of specimens with the physical properties thereof indicated that the inferior metal contained the larger quantity of hydrogen and that the better metal had considerably less hydrogen. Further study of the problem developed that the metal with larger percentages of hydrogen took longer to completely anneal.

My process for improving the physical properties of malleable iron and annealing time of white cast iron is operative for any fuel fired furnace. Where fuel fired furnaces are hereafter referred to, a cupola, air furnace, rotary melting furnace, commercially known as the Brackelsberg furnace, or any other device in which the products of combustion come in contact with the molten white cast iron may be understood. The process is equally operable in any of these methods and I have no desire to restrict myself to the use of any particular form of melting equipment. Moreover, it is operative in cases where two furnaces are used in conjunction with each other, as where the metal is melted in a cupola and further refinement thereof takes place either in an air furnace or in an electric furnace.

The improvement made in the physical properties of malleable iron, which is the product of the white cast iron above referred to, by altering the hydrogen content will be understood by reference to Table I below:

TABLE I

| Specimen | C    | Si   | Tensile | Elonga- | Hydrogen |
|----------|------|------|---------|---------|----------|
|          |      |      |         |         | Percent  |
| 1        | 2.51 | 1.12 | 52216   | 16.0    | 0.00046  |
| 2        | 2.52 | .94  | 52834   | 14.0    | 0.00052  |
| 3        | 2.73 | .92  | 51987   | 16.5    | 0.00050  |
| Average  | 2.59 | .99  | 52346   | 15.5    | 0.00049  |
| 4        | 2.59 | .86  | 45151   | 7.0     | 0.00064  |
| 5        | 2.61 | .97  | 45998   | 6.5     | 0.00080  |
| 6        | 2.52 | 1.10 | 51532   | 7.5     | 0.00060  |
| 7        | 2.71 | .96  | 44727   | 9.5     | 0.00058  |
| Average  | 2.61 | .97  | 44352   | 7.6     | 0.00066  |

For specimens 1, 2 and 3 the table indicates that the average tensile strength is 52,346 pounds per square inch and the average percent elongation is 15.5 for the malleable iron made from the white iron. The average hydrogen content is 0.00049 percent. In specimens 4, 5, 6 and 7 the average hydrogen content is shown as 0.00066 percent. It will be observed that the average reduction in tensile strength for these last four specimens is about 15.0 percent and that the percentage of elongation has been cut approximately in half.

The effect of hydrogen content in white cast iron upon the rate of formation of graphite in the subsequent annealing process can be observed by reference to Table II.

TABLE II

Group 1

| Specimen | Hydrogen | Graphite |
|----------|----------|----------|
|          |          | Percent  |
| 8        | 0.00020  | 0.69     |
| 9        | 0.00025  | 0.54     |
| 10       | 0.00030  | 0.42     |
| 11       | 0.00030  | 0.40     |
| 12       | 0.00046  | 0.38     |
| Average  | 0.00030  | 0.486    |

TABLE II  
Group 2

| Specimen     | Hydrogen<br>by<br>weight | Graphite<br>(after 4<br>hours at<br>900° C.) |
|--------------|--------------------------|----------------------------------------------|
|              | Percent                  | Percent                                      |
| 13.....      | 0.00050                  | 0.085                                        |
| 14.....      | 0.00052                  | 0.18                                         |
| 15.....      | 0.00058                  | 0.037                                        |
| 16.....      | 0.00060                  | 0.515                                        |
| Average..... | 0.00055                  | 0.204                                        |

Group 3

| Specimen     | Hydrogen<br>by<br>weight | Graphite<br>(after 4<br>hours at<br>900° C.) |
|--------------|--------------------------|----------------------------------------------|
|              | Percent                  | Percent                                      |
| 17.....      | 0.00064                  | 0.028                                        |
| 18.....      | 0.00080                  | 0.23                                         |
| 19.....      | 0.00080                  | 0.185                                        |
| 20.....      | 0.00090                  | 0.08                                         |
| 21.....      | 0.00100                  | 0.15                                         |
| 22.....      | 0.00110                  | 0.08                                         |
| Average..... | 0.00084                  | 0.125                                        |

In order to emphasize the difference in result between high and low values of hydrogen Table II is divided into three groups. In Group 1, wherein all values of hydrogen are under 0.00050 percent, the amount of graphite deposited in four hours is uniformly good. In Group 2, with hydrogen between 0.00050 percent and 0.00060 percent, the deposition of graphite is very erratic. In Group 3, which shows hydrogen over 0.00060 percent, the amount of graphite deposited is uniformly low. This suggests that when the hydrogen in white cast iron is much above 0.00050 percent a much longer time for anneal can be expected.

The above tables clearly indicate that very small amounts of hydrogen are definitely detrimental to the strength of the resulting malleable iron and to its annealing rate. One source of hydrogen in white cast iron is the moisture in the air blast. Hydrogen may also be present due to the use of rusty scrap, moisture on the fuel or melting stock, or to the hydrogen in the melting stock itself. The effect of moisture in the air blast on the hydrogen content of the white iron is illustrated in Table III.

TABLE III

|                   | Moisture<br>grains<br>per<br>cu. ft. | Percent<br>hydro-<br>gen<br>by<br>weight | Moisture<br>grains<br>per<br>cu. ft. | Percent<br>hydro-<br>gen<br>by<br>weight | Differ-<br>ence in<br>hydro-<br>gen |
|-------------------|--------------------------------------|------------------------------------------|--------------------------------------|------------------------------------------|-------------------------------------|
| Cupola.....       | 1.30                                 | 0.00024                                  | 2.61                                 | 0.00083                                  | 0.00059                             |
| Air furnace.....  | 1.30                                 | 0.00035                                  | 2.61                                 | 0.00091                                  | 0.00056                             |
| Brackelsberg..... | 1.30                                 | 0.00052                                  | 1.85                                 | 0.00089                                  | 0.00037                             |

The hydrogen concentrations listed in the above table as cupola are the average hydrogen concentrations of the cupola iron used in a duplexing process on two different days in each case, and the moisture content is the average for the same two days for each value. Hydrogen listed as air furnace is the average of the final product of the duplexing operation for the same two days for each amount of moisture. The Brackelsberg results are similarly averages of two days for each moisture concentration. It is evident that variations in the moisture content of the air blast

used with the furnace has a great effect on the amount of hydrogen present. An increase in moisture from 1.30 to 2.61 grains per cubic foot increases the hydrogen in the cupola from 0.00024 percent to 0.00083 percent and in the air furnace from 0.00035 percent to 0.00091 percent. In the Brackelsberg furnace an increase in moisture from 1.30 to 1.85 grains per cubic foot raised the hydrogen from 0.00052 percent to 0.00089 percent.

That the moisture of the air blast is not the only source of hydrogen is indicated by the fact that metal produced by cupola-electric furnace duplexing on a rather damp summer day but from extremely rusty scrap contained 0.00115 percent hydrogen, whereas iron produced from ordinary scrap under the same conditions contained 0.00083 percent.

From Table III moisture contents that would result in about 0.0005 percent hydrogen for the different types of melting furnaces may be readily calculated by linear interpolation. Interpolating in this manner to obtain the moisture content of the air blast for the cupola and air furnace that would result in a hydrogen concentration of not over 0.0005 percent, the figure for the cupola is approximately 1.87 grains per cubic foot and for the air furnace 1.65. Although reasoning based on the mass law and various assumptions as to melting conditions might lead to more complicated methods for interpolating, I feel that for practical purposes such a course is scarcely justified over mere linear interpolation.

It is to be expected that the hydrogen concentration will rise or fall so as to approach equilibrium with the flame of the furnace even though complete equilibrium will not be attained in a commercial process. The limiting moisture content in the air to attain a given desired hydrogen content in the iron is thus to some degree dependent on the hydrogen content of the charge. Since, however, according to my invention the desire is to minimize the hydrogen as far as possible, no harm will result if the blast is dried as far as is commercially feasible.

From what has been said above, it will be clear that any step that will reduce the amount of hydrogen in the white cast iron will improve the physical properties of the resulting malleable iron and also reduce the annealing time for producing the latter. Moreover, any step that will lower the moisture content of the air blast used in melting furnace is of advantage in making malleable iron. The moisture content of the air may be reduced either by refrigeration or by absorption of water by suitable substances such as silica gel or calcium chloride.

In practising my invention I follow the usual procedure for making white iron for conversion into malleable iron with the addition that the moisture content of the air blast supplied to the furnace is reduced by suitable drying means so as to control the hydrogen in the metal.

The terms and expressions which I have employed are used as terms of description and not of limitation, and I have no intention in the use of such terms of excluding any equivalents of the matter described but recognize that various modifications are possible within the scope of the invention.

I claim:

1. A process for improving the physical properties and for shortening the annealing time of malleable iron which comprises melting the iron in a fuel fired furnace and maintaining the hy-

drogen in the melted iron under about 0.0005 percent by controlling the moisture content of the air blast used to support combustion of the fuel.

2. That improvement in the art of making malleable iron which comprises melting the iron in a fuel fired furnace, maintaining the amount of hydrogen in the melted iron below about 0.0005 percent, pouring the metal into molds and annealing the resulting article.

3. A process for improving the physical properties and for shortening the annealing time of malleable iron which comprises melting the iron in a fuel fired furnace and maintaining the moisture content of the air supplied to the fuel under about 1.65 grains per cubic foot to control the hydrogen content of the iron.

4. A process for making malleable iron comprising melting the usual ingredients for white iron in a fuel fired furnace, maintaining the hy-

drogen content of the melt below about 0.0005 percent to improve the physical properties thereof, casting the metal and annealing the casting.

5. A process for making malleable iron comprising melting the usual ingredients for white iron in a fuel fired furnace, maintaining the hydrogen content of the melt below about 0.0005 percent to shorten the time required to anneal the product, casting the metal and annealing the casting for a shorter period than is usual for white cast iron.

6. A process for improving the physical properties and annealing time of malleable iron which comprises melting the iron in an air furnace and maintaining the moisture content of the air supplied to the fuel under about 1.30 grains per cubic foot to control the hydrogen content of the iron.

HARRY A. SCHWARTZ.